

Feb. 18, 1947.

T. GRISWOLD, JR., ET AL

2,416,255

METHOD AND APPARATUS FOR CONDENSING METALLIC VAPORS

Filed March 24, 1945

2 Sheets-Sheet 1



INVENTORS  
Thomas Griswold, Jr.  
BY Thomas H. McConica III

Griswold & Gurdick  
ATTORNEYS

Feb. 18, 1947.

T. GRISWOLD, JR., ET AL

2,416,255

METHOD AND APPARATUS FOR CONDENSING METALLIC VAPORS

Filed March 24, 1945

2 Sheets-Sheet 2



Fig. 2

INVENTORS  
Thomas H. McConica <sup>III</sup>  
BY Thomas Griswold, Jr.

Griswold & Gurdick  
ATTORNEYS

## UNITED STATES PATENT OFFICE

2,416,255

## METHOD AND APPARATUS FOR CONDENSING METALLIC VAPORS

Thomas Griswold, Jr., and Thomas H. McConica, III, Midland, Mich., assignors to The Dow Chemical Company, Midland, Mich., a corporation of Michigan

Application March 24, 1945, Serial No. 584,630

7 Claims. (Cl. 75—66)

1

This invention relates to an improved method and apparatus for condensing metal vapors.

In certain metallurgical processes, a mixture of ore and reducing agent is heated to liberate the metal as a vapor in admixture with other gases, it then being necessary to condense the vapor to convert the metal to usable form. One of the most effective condensing methods consists in passing the vapor mixture into contact with a relatively cool quenching liquid, which serves to shock-chill the metal vapor and to convert it to the liquid or solid state, usually in the form of a solution or suspension in the quenching liquid. The condensed metal is then recovered from the quench liquid by distillation, settling, or other simple means. This quench method is especially advantageous in those processes in which the metal vapor and other gases tend to interact chemically during the condensation step, with consequent loss of valuable metal. Typical instances are met in the recovery of magnesium and of sodium from mixtures with carbon monoxide, such as are formed in the carbothermal processes for making these metals.

In the past, most quench condensing processes have been carried out by means of spray chambers, splash-plate condensers, bubble-towers, and similar absorption apparatus. Unfortunately, such equipment does not always provide a sufficiently drastic quench to arrest completely chemical interaction between metal vapor and accompanying gases, so that part of the metal may never be recovered in usable form. In addition, there may also be some loss of quench liquid by entrainment in the gases exhausted from the condenser. These losses, while not such as to outweigh the advantages of liquid quench condensation, have constituted real practical difficulties for some time.

It is therefore an object of the present invention to provide an improved procedure for condensing a metal vapor by means of a quenching liquid which voids the difficulties mentioned. Another object is to provide apparatus which effects extremely rapid and intimate contact between metal vapor and quench liquid and which minimizes entrainment losses.

In condensing metal vapor in accordance with the invention, the quenching liquid, usually a difficultly volatile molten metal absorbent for the vapor, is disposed in the form of a number of relatively massive continuous streams of liquid flowing in free fall. The vapor mixture from which the metal is to be condensed is then caused to impinge in stream form on the flowing streams

2

of quench liquid. An extreme intimacy of contact between vapor and quench liquid is thus achieved, and instant, virtually complete condensation of the metal takes place. Fixed gases in the vapor mixture pass through the streams of quench liquid and are withdrawn from beyond them.

A more detailed discussion of the invention may be made with reference to the accompanying drawings in which

10 Fig. 1 illustrates, in vertical partial cross-section, one arrangement of apparatus for condensing metal vapors; and

15 Fig. 2 is a cut-away perspective view of the distributor and collector for quench liquid as viewed from the furnace end, showing the plate-like streams of falling liquid.

20 For the sake of example, the process will be described as applied to the production of magnesium by heating a charge mixture of magnesium oxide and carbon to form a vapor mixture of magnesium and carbon monoxide, and condensing the magnesium vapor by means of a lead-magnesium alloy as the quenching fluid.

25 In the equipment illustrated, the magnesium-carbon monoxide vapor mixture is generated in an arc furnace 3 formed of a gas-tight steel shell 4 lined with refractory carbon blocks 5 and having a hearth 6 of broken coke. The furnace is heated electrically by arcs struck between the 30 hearth and graphite electrodes 7 which enter through water-cooled gas-tight glands not shown. Charge mixture is fed in through an upper inlet 8 provided with gas-tight feeding means not illustrated.

35 The vapor mixture leaves the furnace through a narrow-throated orifice 9 formed in a small block 10 of highly refractory material, such as boron carbide. The diameter of the orifice is ordinarily quite small, being usually only a few

40 inches, even for very large furnaces. The orifice block 10 is held by a carbon bushing 11 in a socket in a carbon thrust-block 12 secured in the furnace wall and seated on a steel ring 13 welded to the furnace shell.

45 The vapor mixture liberated in the furnace leaves through the orifice 9 as a high velocity stream and enters a short conduit 14 which leads directly into a thermally insulated chamber 15 in which the magnesium vapor is quenched by impinging on successive plate-like streams 16 of lead-magnesium alloy. The non-condensable carbon monoxide is continuously exhausted from beyond the last stream 16 through a stack 17 leading to a pump 18. Any solid deposit forming 50 in the vapor orifice 9 may be poked loose by an

alloy steel reamer 19 of diameter slightly less than that of the orifice. This rod is mounted slidably opposite the orifice in a gland 20 welded through a cover flange 21 on the end of the quench chamber.

The lead-magnesium quench alloy is maintained under inert gas protection in a closed insulated reservoir 22 provided with heat exchangers not shown for maintaining the alloy at a temperature below 650° C. This liquid is continuously forced by a pump 23 driven by a motor 24 through an insulated line 25 into a distributing box 26 mounted in the quench chamber 15 above the path of the vapor issuing from the orifice 9. In the bottom of the box 26, a series of parallel elongated rectangular slots 27 are cut in a direction perpendicular to the path of the magnesium vapor stream, these slots extending across almost the entire width of the quench chamber. The alloy delivered to the box 26 flows through the slots 27 and falls freely across the issuing furnace vapor in the form of plate-like streams 16 of sufficient thickness to constitute practically unbroken curtains of moving metal. These streams fall into a collecting basin 28, which is formed in the chamber 15 directly under the distributing box 26 and below the path of the furnace vapor stream, and are returned to the reservoir 22 through an insulated drain 29. Part of the quench liquid containing condensed magnesium is withdrawn continually from the reservoir by a pump 30 driven by a motor 31 and is circulated through a pipe 32 to a system, not shown, for distilling magnesium from the alloy, from which the magnesium-depleted liquid is returned for re-use by a pipe 33.

In operation of the apparatus, the vapor stream of magnesium and carbon monoxide issues from the orifice 9 at considerable velocity, usually at least several hundred feet per second, and impinges on the falling curtains 16 of quench alloy. The gaseous stream forces its way successively through each of the curtains in an extremely short period of time, and during such passage is thoroughly scrubbed by the falling alloy. The magnesium vapor is effectively condensed and absorbed by the alloy, being thus separated from the carbon monoxide, which is exhausted through the stack 17. The enriched alloy returns to the reservoir 22, from which it may be withdrawn to the magnesium recovery step.

In the apparatus of the drawing, the slots 27 must be wide enough that the streams of quench liquid falling through them are sufficiently massive that there is no tendency for them to become discontinuous, i. e., to break up into a shower of discrete drops, under the action of the impinging vapor stream. In general, a slot width of at least 0.5 inch, and preferably 1.0 inch or more, is required when the height of free fall of the quench liquid is 2 or 3 feet.

While, according to the invention, the quench liquid is preferably formed into massive plate-like streams by means of slots, as illustrated, it is also possible to dispose the liquid in the form of rod-like streams, as by providing several series of holes, instead of slots, in the bottom of the distributing box 26. These rod-like streams, which should be of diameter sufficient that they do not break up into a rain of drops during their fall, are best spaced closely in staggered array so that there is no possibility that the vapor stream issuing from the furnace can find its way through the quench chamber without passing into intimate contact with several of the liquid streams.

The impingement of a high-velocity stream of gas and vapor on continuous streams of flowing quench liquid in the manner of the invention offers a number of advantages not shared by quenching procedures used heretofore:

1. The duration of actual contact between the vapor stream and the quench liquid is exceedingly short, so that interaction between the vapor and the fixed gas present, or between the gas and the quench liquid, is at a minimum.

2. Every portion of the gas is withdrawn from contact with the quench liquid immediately upon being freed of vapor, and on the opposite side of the streams from that of the furnace outlet. The fixed gas never tends to build up in the condenser, diluting the incoming vapor stream or blanketing it from effective contact with the quench liquid.

3. The surface of the quench streams is constantly renewed so that there is little local overheating or saturation of any part of the condensing area.

4. The streams of quench liquid present an ever-shifting surface to the incoming gas. Channelling of the vapor stream through the condenser, with consequent inefficiency of gas-liquid contact and loss of uncondensed vapor, does not occur to any degree.

5. Inasmuch as the flowing streams of quench liquid are massive and continuous, in contrast to a spray or a rain of drops, there is little tendency for entrainment of the quench liquid in the exhaust gas.

6. Practically all inner surfaces of the quench chamber are constantly wetted by the flowing liquid, so that foreign particles carried by the incoming vapor stream are washed away. Formation of troublesome deposits is largely prevented.

As a result of these and other considerations, exceptionally high quenching efficiencies are realized and operating difficulties are held at a minimum.

While the invention has been described with particular reference to the manufacture of magnesium, it is equally applicable to the quenching of sodium vapors in lead-sodium alloys. Further, so far as known, it may advantageously be applied to the condensation step of any metallurgical process in which a mixture of a reducible compound of a volatilizable metal and a reducing agent is heated to liberate metal vapor, which must then be condensed. Still other applications of the invention will doubtless occur to those familiar with the general field.

What is claimed is:

1. In a metallurgical condensation process in which a mixture of a metal vapor and a fixed gas is passed into intimate contact with a quenching liquid to condense the vapor, the improved procedure which comprises disposing the quenching liquid as a horizontal series of plate-like massive streams flowing vertically downward in free fall, causing the vapor mixture to impinge horizontally in stream form on the first liquid stream of the series and thence to pass into contact with each of the succeeding streams, whereby the vapor is substantially all condensed, and continuously withdrawing fixed gas beyond the last liquid stream of the series.

2. A process according to claim 1 in which the quenching liquid is a difficultly volatile molten metal absorbent for the vapor.

3. A process according to claim 1 in which the metal vapor is magnesium and the quenching liquid is a lead-magnesium alloy.

4. A process according to claim 1 in which the

metal vapor is sodium and the quenching liquid is a lead-sodium alloy.

5. A metallurgical process which comprises: heating a mixture of a reducible compound of a volatilizable metal and a reducing agent to a temperature sufficient to form metal vapor in a confined zone provided with a restricted outlet through which the liberated vapor issues as a horizontal stream, causing a quenching liquid for the metal vapor to flow vertically downward across the path of the issuing vapor stream in the form of a horizontally extending series of plate-like massive streams flowing in free fall, whereby the metal vapor impinges on the streams of quenching liquid and is condensed, withdrawing uncondensed gas from beyond the last of the liquid streams, and collecting the quenching liquid after its passage across the vapor stream and recovering metal therefrom.

6. Metallurgical apparatus for condensing metal vapor in a quenching liquid comprising, in combination with a source of metal vapor and a reservoir for quenching liquid: a gas-liquid contact chamber in communication with the vapor source through a restricted orifice; a distributing box for quenching liquid mounted in the chamber above the path of vapor issuing from the orifice, the bottom of the box having therein a series of parallel slots disposed transversely to the path of the issuing vapors, each slot being sufficiently wide that quench liquid falls therethrough as a plate-like massive stream; liquid collecting means for receiving liquid falling from the box mounted in the chamber under the distributing box and below the path of the vapor issuing from the orifice; and circulating means for withdrawing liquid from the reservoir and supplying it to the distributing box and for withdrawing liquid from the collecting means and returning it to the reservoir.

40

7. Metallurgical apparatus comprising: a metal-vapor generating furnace having a restricted vapor outlet; a quench condenser in communication with the furnace through the outlet; a source of quenching liquid; distributing means within the condenser for disposing the quenching liquid across the path of vapor issuing from the furnace outlet in the form of a horizontally-extending series of parallel plate-like massive streams, each flowing vertically downward; collecting means within the condenser for receiving the streams of quench liquid; circulating means for conveying quenching liquid from its source to the distributing means and for returning it from the collecting means to the source; and exhaust means for removing uncondensed gas from the quench chamber at a point on the opposite side of the liquid streams from that of the furnace outlet.

THOMAS GRISWOLD, JR.  
THOMAS H. McCONICA, III.

## REFERENCES CITED

The following references are of record in the file of this patent:

## UNITED STATES PATENTS

| Number    | Name         | Date          |
|-----------|--------------|---------------|
| 967,135   | Lachance     | Aug. 9, 1910  |
| 879,149   | Cunningham   | Feb. 18, 1908 |
| 2,031,437 | Vincent, Jr. | Feb. 18, 1936 |
| 902,535   | Johnson      | Oct. 27, 1908 |
| 2,238,909 | McConica     | Apr. 22, 1941 |

## FOREIGN PATENTS

| Number  | Country | Date         |
|---------|---------|--------------|
| 121,752 | British | Jan. 9, 1919 |